

Dec. 12, 1939.

K. ERDMANN

2,183,392

METHOD OF CONVERTING MAGNESIUM DUST INTO COMPACT METALLIC MAGNESIUM

Filed Aug. 2, 1938



Konrad Erdmann  
INVENTOR

By  
Brown, Critchlow & Flick  
his attorneys

## UNITED STATES PATENT OFFICE

2,183,392

## METHOD OF CONVERTING MAGNESIUM DUST INTO COMPACT METALLIC MAGNESIUM

Konrad Erdmann, Radenthein, Germany, assignor to American Magnesium Metals Corporation, Pittsburgh, Pa., a corporation of Delaware

Application August 2, 1938, Serial No. 222,624  
In Austria August 16, 1937

## 5 Claims. (Cl. 75—67)

This invention relates to a process for the conversion of magnesium dust into compact magnesium metal.

The object of the present invention is to provide a simple and economical method for recovering compact metal from magnesium dust by vaporization of the magnesium and re-condensation of the vapors.

A further object is to enable the metal vapors to be disengaged practically free from dusty impurities.

In the course of the electrothermic production of magnesium metal by smelting magnesium oxide or prime materials containing magnesium oxide, with the aid of carbon, there is obtained in the first stage of operation, on the condensing of the magnesium disengaged in the form of vapor, as an intermediate product a dusty condensate containing 50 to 90 percent of metallic magnesium while the remainder substantially consists of magnesium oxide and carbon, all these constituents being contained in the dusty condensate in a state of extremely fine division. The magnesium is recovered from this dust, in a second stage of operation, by distillation or sublimation.

If in this second stage the magnesium dust were to be subjected, just as it is, to distillation or sublimation there would result, as the final product, metal heavily contaminated with non-volatile impurities, since owing to the very small size of the said impurities the disengaged magnesium vapors entrain a major portion thereof with them. It was therefore necessary to have recourse to the usual expedient of making the dust into compacted bodies before further treatment which was done by commixing the dust with non-volatile additions (such as carbon and magnesium oxide), impasting the mixture with the aid of hydrocarbon oil and driving off the oil preferably at a temperature at which a part of the oil will crack to form a firmly coherent coke matrix.

Later it has been found that it would be simpler and more economical to form the pulverulent mixture for the purpose in question into compacted bodies by molding the same under high pressure, preferably in an atmosphere of gas indifferent to magnesium, without the addition of any binding material. However, the briquettes or the like produced in this manner are of inadequate strength, so that particularly in the carrying out of the distillation or sublimation by passing the briquettes through a furnace in an uninterrupted working operation fine particles become detached from the briquettes by rubbing, and pass together with the vapors into the con-

denser, which trouble increases rapidly with the progressive driving off of the magnesium, since the remainder of the pieces, the skeleton so to speak, gets more and more light and porous. This difficulty becomes particularly troublesome in connection with the working up of dust very rich in magnesium. Attempts undertaken with the view of enhancing the strength of the compacted bodies by considerably increasing the amount of non-volatile substances by means of additions ensuring the continued stability of the pieces during and after the final distillation operation have been made in vain; when transforming the dust into compacted bodies by simply molding the same under high pressure without having recourse to the use of other expedients for increasing the coherence no appreciable improvement could be achieved either by the admixing of finely divided carbon such as soot, or by the admixing of finely divided magnesium oxide to the material to be briquetted.

According to the present invention, the described drawback is overcome by adding to the material to be formed into compacted bodies under high pressure without having recourse to other expedients for increasing the coherence, particularly to the addition of binding material, finely ground residues left behind as the non-volatile remainder in the distilling out or subliming out of the magnesium from such bodies in a previous working operation. It has surprisingly transpired that, as a result of admixing such residues, the strength of the molded bodies is suddenly and greatly improved, as may be seen from the following comparative table:

| Material briquetted                                               | Crushing strength in kgs./cm. <sup>2</sup> |                    |
|-------------------------------------------------------------------|--------------------------------------------|--------------------|
|                                                                   | Before distillation                        | After distillation |
| Dust (containing 32% of Mg) by itself.....                        | 113                                        | 0                  |
| Same dust + 30% of dead burned magnesite.....                     | 62                                         | 0                  |
| Same dust + 30% of soot.....                                      | 90                                         | 0                  |
| Same dust + 30% of anthracite.....                                | 50                                         | 0                  |
| Same dust + 30% of bituminous coal coke.....                      | 15                                         | 0                  |
| Same dust + 30% of residues from preceding distillation runs..... | 137                                        | 39                 |

For putting the process into practice, the residue left behind as the non-volatile remainder in a preceding working operation, e. g. distillation operation, is ground and then sifted so as to obtain a fine meal fraction containing 95% of particles smaller than 0.01 mm., whereas the coarser particles are withdrawn. The fine meal fraction

is intimately mixed with the magnesium dust to be worked up and the mixture then molded under a high pressure, for instance of the order of 1000 kg./cm.<sup>2</sup>, to be formed into bodies of a diameter between 30 and 50 mm. The amount of the residue due to be introduced depends on the magnesium content of the dust. It has proved suitable to adjust this amount in such a manner that the metal content in the compacted body does not exceed 40%.

The whole series of operations has to be carried out under exclusion of air, preferably in an inert atmosphere, for instance hydrogen.

The vapor cooled may be condensed either to a liquid deposit, which sets to reguline metal, or directly from the vapor phase to a solid deposit capable of coalescing under heat.

The drawing shows diagrammatically an apparatus adapted for carrying out the process by way of example.

The spent residue leaving the plant 1 in which the preceding working operation has taken place passes through the condenser 2 into a lock-chamber 3 delivering 70% of the amount collected into trucks to be taken to the waste dump. The remainder is carried by a suitable conveyor 5a to a stock vessel 4, whence the material is delivered in properly adjusted portions, by a conveyor 5b to the ball mill 6 provided with a sifter. The material that fails to pass through the screen drops into a suitable receptacle, while the material passing through the screen is taken by a conveyor 5c into the head of a mixing bunker 7 into which at the same time the required amount of magnesium dust to be worked up is introduced by a conduit 8 so as to bring together the same there with the finely ground residue. The mixture is fed into a briquetting press 9 of the known type used in briquetting lignite, whence the compacted bodies are passed, by a suitable conveying device, to the distilling furnace.

I claim:

1. Process of converting magnesium dust into compact metallic magnesium by extracting the magnesium content therefrom by means of vaporization and subsequent re-condensation of the vapor, which process comprises mixing the magnesium dust with ground residue left behind as the non-volatile remainder in a previous operation involving vaporization of magnesium from magnesium dust, making the mixture into compacted bodies under high pressure without the addition of binding material, subjecting the briquettes thus obtained to a heat treatment to drive out the magnesium in the form of vapor, and condensing the vapor evolved.

2. A process of converting magnesium dust into compact metallic magnesium by extracting the magnesium content therefrom by means by vaporization and subsequent re-condensation of the

vapor, which process comprises mixing the magnesium dust with ground residue left behind as the non-volatile remainder in a preceding operation involving vaporization of magnesium from magnesium dust, forming the mixture into compacted bodies under high pressure without having recourse to other expedients for increasing the coherence, and then interposing the compacted bodies thus obtained as resistor between the poles in an electric furnace to drive out the magnesium in the form of vapor, and condensing the vapor.

3. Process of converting magnesium dust into compact metallic magnesium by extracting the magnesium content therefrom by means of vaporization and subsequent re-condensation of the vapor, which process comprises mixing the magnesium dust with ground residue left behind as the non-volatile remainder in the extracting of the magnesium in a previous operation involving vaporization of magnesium from magnesium dust and molding the mixture into strongly compacted bodies without the addition of binding material, both these operations being carried out under exclusion of air, and then subjecting the briquettes thus obtained to a heat treatment to drive out the magnesium in the form of vapor, and condensing the vapor evolved.

4. Process of converting magnesium dust into compact metallic magnesium by extracting the magnesium content therefrom by means of vaporization and subsequent re-condensation of the vapor, which process comprises mixing the magnesium dust with finely ground spent residue left behind as the non-volatile remainder in a preceding operation involving vaporization of magnesium from magnesium dust, briquetting the mixture under high pressure without the addition of binding material, both these operations being carried out in an atmosphere of inert gas, and then heating the briquettes thus obtained to vaporize the magnesium, and condensing the vapor evolved to a liquid deposit which sets to reguline metal.

5. Process of converting magnesium dust into compact metallic magnesium by extracting the magnesium content therefrom by means of vaporization and subsequent re-condensation of the vapor, which process comprises mixing the magnesium dust with finely ground spent residue left behind as the non-volatile remainder in a preceding operation involving vaporization of magnesium from magnesium dust, molding the mixture under high pressure into compacted bodies without the addition of binding material, heating the briquettes thus obtained to vaporize the magnesium, and condensing the vapor evolved directly from the vapor phase to a solid deposit capable of coalescing under heat.

KONRAD ERDMANN.

60